



US005879867A

# United States Patent [19]

Zengerle et al.

[11] Patent Number: **5,879,867**[45] Date of Patent: **Mar. 9, 1999**

[54] **SILVER HALIDE LIGHT-SENSITIVE ELEMENT**

[75] Inventors: **Paul L. Zengerle**, Rochester; **Gary N. Barber**, Penfield; **Leslie Gutierrez**, Rochester, all of N.Y.

[73] Assignee: **Eastman Kodak Company**, Rochester, N.Y.

[21] Appl. No.: **916,240**

[22] Filed: **Aug. 22, 1997**

[51] Int. Cl.<sup>6</sup> ..... **G03C 7/36**; G03C 7/388

[52] U.S. Cl. ..... **430/505**; 430/546; 430/557

[58] Field of Search ..... 430/546, 557,  
430/505

## [56] References Cited

### U.S. PATENT DOCUMENTS

|           |         |                  |         |
|-----------|---------|------------------|---------|
| 2,322,027 | 6/1943  | Jelley et al.    | 430/546 |
| 2,787,544 | 4/1957  | Godowsky et al.  | 430/546 |
| 2,801,170 | 7/1957  | Vittum et al.    | 430/546 |
| 3,676,141 | 7/1972  | Hara et al.      | 430/377 |
| 3,973,968 | 8/1976  | Fujiwhara et al. | 430/389 |
| 4,057,432 | 11/1977 | Fujiwhara et al. | 430/389 |
| 4,221,860 | 9/1980  | Hirose et al.    | 430/557 |
| 4,269,936 | 5/1981  | Arai et al.      | 430/557 |
| 4,314,023 | 2/1982  | Kojima et al.    | 430/557 |
| 4,327,175 | 4/1982  | Toda et al.      | 430/546 |
| 4,404,274 | 9/1983  | Arai et al.      | 430/557 |
| 4,456,681 | 6/1984  | Kadowaki et al.  | 430/557 |
| 4,581,324 | 4/1986  | Wolff et al.     | 430/557 |

|           |         |                  |         |
|-----------|---------|------------------|---------|
| 4,748,107 | 5/1988  | Umemoto et al.   | 430/551 |
| 4,770,985 | 9/1988  | Takada et al.    | 430/557 |
| 5,100,771 | 3/1992  | Mihayashi et al. | 430/557 |
| 5,173,398 | 12/1992 | Fukazawa et al.  | 430/546 |
| 5,358,831 | 10/1994 | Bagchi et al.    | 430/546 |

### FOREIGN PATENT DOCUMENTS

0 374 837 B1 3/1995 European Pat. Off. .

Primary Examiner—Richard L. Schilling  
Attorney, Agent, or Firm—Andrew J. Anderson

[57]

### ABSTRACT

A silver halide light sensitive photographic element is disclosed comprising a support bearing at least one yellow image forming hydrophilic colloid layer comprising yellow image dye forming couplers, at least one hydrophilic colloid layer immediately adjacent to the yellow image forming layer, and at least one adjacent cyan or magenta image forming hydrophilic colloid layer comprising cyan or magenta image dye forming couplers; wherein the yellow image forming layer is substantially free of high boiling permanent solvent, any immediately adjacent hydrophilic colloid layers and the adjacent image forming layer are substantially free of high boiling permanent solvents having a logP value of less than about 5.5, and the adjacent image forming layer contains a high boiling permanent solvent having a logP value of at least about 5.5. The photographic elements exhibit good yellow image dye light stability, which is not degraded by the presence of relatively high logP value solvents in immediately adjacent hydrophilic colloid layers and other adjacent imaging layers.

**17 Claims, No Drawings**

## SILVER HALIDE LIGHT-SENSITIVE ELEMENT

### TECHNICAL FIELD

This invention relates generally to the field of silver halide light sensitive elements, and in particular to photographic elements having at least one yellow imaging layer which is essentially free of permanent high boiling coupler solvent and an adjacent imaging layer containing relatively hydrophobic coupler solvents. In a particular aspect it relates to motion picture print films.

### BACKGROUND OF THE INVENTION

Various techniques are known for dispersing hydrophobic photographically useful compounds such as photographic couplers into photographic element layer coating compositions comprising hydrophilic colloids.

Photographic dye forming couplers, as well as other hydrophobic photographically useful compounds, are typically incorporated into a hydrophilic colloid layer of a photographic element by first forming an aqueous dispersion of the couplers and then mixing such dispersion with the layer coating solution. An organic solvent is typically used to dissolve the coupler, and the resulting organic solution is then dispersed in an aqueous medium to form the aqueous dispersion.

The organic phase of these dispersions frequently includes high boiling or permanent organic solvents, either alone or with low boiling or water miscible solvents which are removed after dispersion formation. Permanent high boiling solvents have a boiling point sufficiently high, generally above 150° C. at atmospheric pressure, such that they are not evaporated under normal dispersion making and photographic layer coating procedures. Permanent high boiling coupler solvents are primarily used in the conventional "oil-protection" dispersion method whereby the organic solvent remains in the dispersion, and thereby is incorporated into the emulsion layer coating solution and ultimately into the photographic element.

The conventional "oil in water" dispersion method for incorporating hydrophobic couplers is described, e.g., in U.S. Pat. No. 2,322,027 by Jelly and Vittum. In such conventional process, the coupler is dissolved in a high boiling water immiscible solvent, mixed with aqueous gelatin, and dispersed using a colloid mill or homogenizer. The presence of the high boiling solvent provides a stable environment for the hydrophobic coupler, as well as generally increasing the reactivity of the coupler upon photographic processing.

U.S. Pat. No. 2,801,170 of Vittum et al. discloses preparing separate dispersions of a coupler and a high boiling point solvent and mixing the two dispersions with a silver halide emulsion. U.S. Pat. No. 2,787,544 of Godowsky et al. discloses a method of making mixed packet photographic systems. A dispersion of high boiling point solvent is mixed with a dispersion of coupler. Both these processes help prevent crystallization of the coupler prior to layer coating by keeping the solvent and the coupler separate until just prior to coating, while providing solvent in the coated layer to enhance coupler reactivity in the photographic element.

While the presence of high boiling solvents in certain coupler dispersions in photographic elements is frequently desirable to provide, e.g., adequate coupler reactivity upon photographic processing, lower thermal yellowing, modified dye hues, enhanced dye dark stability, and reduced

crystallization, there are also certain advantages which may result from the substantial elimination of high boiling permanent solvent from a photographic element imaging layer. U.S. Pat. No. 5,173,398, e.g., discloses photographic elements with coupler-containing layers having substantially no high boiling solvent. Alternative methods for delivering hydrophobic materials, such as color couplers, to aqueous based photographic compositions without using high boiling solvents are well known in the art. Such techniques involve, e.g., deposition of the couplers from basic aqueous solutions or volatile low boiling or water miscible organic auxiliary solvents followed by removal of the auxiliary solvent by evaporation or washing, mechanical dispersion methods wherein solid compounds are directly dispersed in an aqueous composition, and latex loading methods wherein, e.g., a coupler is loaded into a latex polymer by mixing a solution of the coupler in a low boiling or water miscible organic solvent with an aqueous suspension of the latex followed by removal of the solvent. Minimizing the amount of permanent coupler solvent coated in a photographic element is useful, e.g., for reducing the coated thickness of photographic layers. Reductions in coupler solvent level also afford concomitant reductions in gelatin level which leads to further reductions in coated dry thickness. Layer thinning is advantageous for reasons such as improved image sharpness due to reduced light scattering during exposure and increased developability due to shorter diffusion paths through the multilayer structure. This increase in developability can lead to lower silver and/or coupler coated levels, hence lower materials cost.

Additional advantageous properties may also be associated with the absence of coupler solvent in a particular layer. The light stability for yellow image dyes formed in an exposed and processed photographic element, e.g., may be significantly improved where the yellow dyes are formed in a photographic layer which is substantially free of organic solvents, such as disclosed in concurrently filed, commonly assigned, copending applications U.S. Ser. No. 08/916,882 (Kodak Docket No. 75629AJA) and U.S. Ser. No. 08/916,842 (Kodak Docket No. 76462AJA) the disclosures of which are incorporated by reference herein. It may be desirable to include organic solvents in cyan or magenta image dye forming layers while eliminating such solvent from the yellow dye forming layer, however, as coupler solvent reduction can frequently result in disadvantageous features in such layers such as reducing the reactivity of the dispersed cyan or magenta dye forming coupler to a level too low to produce desired dye density upon processing of the photographic material, higher thermal yellowing, lower dye dark stability, and increased crystallization. In balancing such requirements and desired features in a color photographic element, it thus may be desirable to include organic solvents in some image forming layers, while eliminating solvents from other image forming layers.

It has been found that the advantageous improvement in yellow image dye light stability associated with the removal of solvent from a yellow image forming layer of a photographic element may be degraded when an adjacent cyan or magenta imaging layer contains an organic solvent. It would be desirable to provide a silver halide photographic element which contains a yellow image forming layer which is substantially free of high boiling organic solvent and an adjacent cyan or magenta image forming layer which contains organic solvent in which the yellow image dye light stability is not significantly degraded by the presence of the solvent coated in an adjacent imaging layer.

### SUMMARY OF THE INVENTION

One embodiment of the invention comprises a silver halide light sensitive photographic element comprising a

support bearing at least one yellow image forming hydrophilic colloid layer comprising yellow image dye forming couplers, at least one hydrophilic colloid layer immediately adjacent to the yellow image forming layer, and at least one adjacent cyan or magenta image forming hydrophilic colloid layer comprising cyan or magenta image dye forming couplers; wherein the yellow image forming layer is substantially free of high boiling permanent solvent, any immediately adjacent hydrophilic colloid layers and the adjacent image forming layer are substantially free of high boiling permanent solvents having a logP value of less than about 5.5, and the adjacent image forming layer contains a high boiling permanent solvent having a logP value of at least about 5.5.

In a preferred embodiment, a silver halide light sensitive photographic element is described comprising a support bearing in sequential order on one side thereof at least one yellow image forming hydrophilic colloid layer comprising a blue-sensitive silver halide emulsion and yellow image dye forming coupler, a hydrophilic colloid layer immediately adjacent to the yellow image forming layer, at least one cyan image forming hydrophilic colloid layer comprising red-sensitive silver halide emulsion and cyan image dye forming coupler, and at least one magenta image forming hydrophilic colloid layer comprising green-sensitive silver halide emulsion and magenta image dye forming coupler; wherein the yellow image forming layer is substantially free of high boiling permanent solvent, the hydrophilic colloid layer immediately adjacent the yellow image forming layer and the cyan image forming layer are substantially free of high boiling permanent solvents having a logP of less than about 5.5, and the cyan image forming layer contains a high boiling permanent solvent having a logP value of at least about 5.5.

## ADVANTAGES

The photographic elements of the invention employing substantially solvent-free yellow imaging layers exhibit good yellow image dye light stability, which is not degraded by the presence of relatively high logP value solvents in immediately adjacent hydrophilic colloid layers and other adjacent imaging layers.

## DETAILED DESCRIPTION

The photographic elements of the invention comprise at least one yellow image forming hydrophilic colloid layer comprising yellow image dye forming couplers, which layer is substantially free of high boiling permanent solvent. The term "high boiling permanent solvent" as used herein refers to those coupler solvents which have conventionally been employed in the photographic industry, such solvents typically being water immiscible and having a boiling point of above 150° C. For the purposes of this invention, "substantially free of high boiling permanent solvent", "no-solvent", and like terms are intended to denote the absence of permanent organic solvents beyond trace or impurity levels. Yellow image forming layers in accordance with the invention which are substantially free of high boiling permanent solvents preferably contain 1.0 wt % or less relative to the total amount of yellow coupler in the layer, more preferably less than 0.5 wt %, and most preferably less than 0.1 wt % high boiling permanent solvent relative to the amount of yellow coupler. Such no-solvent dispersions of yellow image forming couplers have been found to provide improved performance with respect to yellow image dye fading problems in exposed and processed photographic

elements in comparison to use of yellow coupler dispersions having significant permanent solvent levels.

Couplers that form yellow dyes upon reaction with oxidized color developing agent and which are useful in elements of the invention are described in such representative patents and publications as: U.S. Pat. Nos. 2,875,057; 2,407,210; 3,265,506; 2,298,443; 3,048,194; 3,447,928 and "Farbkuppler—Eine Literature Ubersicht," published in Agfa Mitteilungen, Band III, pp. 112-126 (1961). Such couplers are typically open chain ketomethylene compounds. Also preferred are yellow couplers such as described in, for example, European Patent Application Nos. 482,552; 510,535; 524,540; 543,367; and U.S. Pat. No. 5,238,803.

15 Typical preferred yellow couplers are represented by the following formulas:



wherein  $R_1$ ,  $R_2$ ,  $Q_1$  and  $Q_2$  each represent a substituent;  $X$  is hydrogen or a coupling-off group;  $Y$  represents an aryl group or a heterocyclic group;  $Q_3$  represents an organic residue required to form a nitrogen-containing heterocyclic group together with the illustrated nitrogen atom; and  $Q_4$  represents nonmetallic atoms necessary to form a 3- to 5-membered hydrocarbon ring or a 3- to 5-membered heterocyclic ring which contains at least one hetero atom selected from N, O, S, and P in the ring. Preferred couplers are of YELLOW-1 and YELLOW-4 wherein  $Q_1$  and  $Q_2$  each represent an alkyl group, an aryl group, or a heterocyclic group, and  $R_2$  represents an aryl or alkyl group, including cycloalkyl and bridged cycloalkyl groups, and more preferably a tertiary alkyl group. Particularly preferred yellow couplers for use in elements of the invention are represented by YELLOW-4, wherein  $R_2$  represents a tertiary alkyl group and  $Y$  represents an aryl group, and  $X$  represents an aryloxy or N-heterocyclic coupling-off group. The elements of the invention are particularly useful in combination with yellow couplers of the above formulas wherein  $X$  represents a nitrogen-containing heterocyclic coupling-off group such as disclosed in concurrently filed, commonly assigned, copending application U.S. Ser. No. 08/916,842 (Kodak Docket No. 76462AJA) incorporated by reference above.

The dispersion of yellow image forming couplers for use in the invention can be prepared by dissolving the couplers in a low boiling or partially water soluble auxiliary organic solvent, or by melting the couplers. The resulting liquid organic phase may then be mixed with an aqueous gelatin solution, and the mixture is then passed through a mechani-

cal mixing device suitable for high shear or turbulent mixing generally suitable for preparing photographic emulsified dispersions, such as a colloid mill, homogenizer, microfluidizer, high speed mixer, ultrasonic dispersing apparatus, blade mixer, device in which a liquid stream is pumped at high pressure through an orifice or interaction chamber, Gaulin mill, blender, etc., to form small particles of the organic phase suspended in the aqueous phase. More than one type of device may be used to prepare the dispersions. The auxiliary organic solvent, if present, may then be removed by evaporation, noodle washing, or membrane dialysis. If not removed prior to coating in a photographic element layer, partially water soluble auxiliary organic solvents may diffuse throughout the hydrophilic colloid layers of the element, and be removed during photographic processing. The dispersion particles preferably have an average particle size of less than 2 microns, generally from about 0.02 to 2 microns, more preferably from about 0.02 to 0.5 micron. These methods are described in detail in U.S. Pat. Nos. 2,322,027, 2,787,544, 2,801,170, 2,801,171, 2,949, 360, and 3,396,027.

Examples of suitable auxiliary solvents which can be used include: ethyl acetate, isopropyl acetate, butyl acetate, ethyl propionate, 2-ethoxyethylacetate, 2-(2-butoxyethoxy) ethyl acetate, triethylcitrate, dimethylformamide, 2-methyl tetrahydrofuran, triethylphosphate, cyclohexanone, butoxyethyl acetate, methyl isobutyl ketone, methyl acetate, 4-methyl-2-pentanol, diethyl carbitol, 1,1,2-trichloroethane, 1,2-dichloropropane, and the like. Preferred auxiliary solvents include ethyl acetate and 2-(2-butoxyethoxy) ethyl acetate.

The aqueous phase of the coupler dispersions preferably comprise gelatin as a hydrophilic colloid. This may be gelatin or a modified gelatin such as acetylated gelatin, phthalated gelatin, oxidized gelatin, etc. Gelatin may be base-processed, such as lime-processed gelatin, or may be acid-processed, such as acid processed ossein gelatin. Other hydrophilic colloids may also be used, such as a water soluble polymer or copolymer including, but not limited to poly(vinyl alcohol), partially hydrolyzed poly(vinylacetate-co-vinyl alcohol), hydroxyethyl cellulose, poly(acrylic acid), poly(1-vinylpyrrolidone), poly(sodium styrene sulfonate), poly(2-acrylamido-2-methane sulfonic acid), polyacrylamide. Copolymers of these polymers with hydrophobic monomers may also be used.

The photographic elements of the invention further comprise at least one hydrophilic colloid layer immediately adjacent to the yellow image forming layer and at least one adjacent image forming hydrophilic colloid layer comprising cyan or magenta image dye forming couplers, wherein the immediately adjacent hydrophilic colloid layers and the adjacent image forming layer are substantially free of high boiling solvents having a logP value of less than about 5.5, and the adjacent image forming layer contains a high boiling solvent having a logP value of at least about 5.5. The term "adjacent image forming layer" refers to a separate image forming layer of the element which is distinct from the solvent-free yellow image forming layer of the invention. The term "immediately adjacent hydrophilic colloid layer" refers to any hydrophilic layer which is coated contiguously on either side of the yellow image forming layer. Such immediately adjacent layers may comprise, e.g., antihalation layers, interlayers, subbing layers, etc. Alternatively, the adjacent image forming layer may itself comprise the immediately adjacent layer.

The log P parameter is a well-known measurement of the solubility of a compound in aqueous liquids compared to its

solubility in a nonpolar organic solvent (octanol). The log P parameter is further described, along with data for organic compounds, in C. Hansch & T. Fujita, *J. Am. Chem. Soc.*, 86, 1616-25 (1964) and A. Leo & C. Hansch, *Substituent Constants for Correlation Analysis in Chemistry and Biology*, Wiley, New York (1979), the disclosures of which are incorporated herein by reference. If the log P of the organic solvent contained in the adjacent imaging layer is less than about 5.5, it will be relatively too hydrophilic to sufficiently prevent the solvent from migrating through the hydrophilic colloid layers of the invention and degrading the light stability of the yellow image dyes formed upon exposure and processing of the photographic elements of the invention.

An adjacent imaging layer (i.e., a layer other than the substantially solvent free yellow image forming layer) of the photographic elements of the invention comprises a high boiling permanent solvent having a logP of at least about 5.5. Such adjacent image forming layers may be, e.g., cyan or magenta image forming layers comprising cyan or magent dye forming couplers. Representative high log P permanent solvents for use in accordance with the invention include, e.g., relatively high logP compounds selected from esters of dicarboxylic acids, such as phthalic acid and sebacic acid, esters of phosphoric acid and benzoic acid, substituted phenols, alcohols, amides, amines, and the like.

Solvents having a high log P in accordance with preferred embodiments of the invention may be so highly hydrophobic that it is difficult to measure their water solubility using standard techniques. Such compounds may have a solubility in water, e.g., of less than 1.0  $\mu\text{g}/\text{mL}$ . In such cases,  $\text{LogP}_{(\text{calc})}$  is a useful means to characterize their hydrophobicity, where  $\text{LogP}_{(\text{calc})}$  is the logarithm of the value of the octanol/water partition coefficient (P) of the compound calculated using MedChem, version 3.54, a software package available from the Medicinal Chemistry Project, Pomona College, Claremont, Calif.  $\text{LogP}_{(\text{calc})}$  is a parameter which is highly correlated with measured water solubility for compounds spanning a wide range of hydrophobicity.

Preferred high log P solvents and their calculated log P values include: dicyclohexylphthalate (6.81), bis(2-ethylhexyl)phthalate (8.92), dinonylphthalate (9.98), didecylphthalate (11.04), diundecylphthalate (12.10), didodecylphthalate (13.16), trihexylphosphate (6.70), tricyclohexylphosphate (6.70), tricresylphosphate (6.58), tris(2-ethylhexyl)phosphate (9.49), trioctylphosphate (9.49), dipropylundecanamide (6.05), dibutylundecanamide (7.10), N-2-ethylhexylundecanamide (7.79), dibutylsebacate (5.98), bis(2-ethylhexyl)sebacate (10.22), di-t-pentylphenol (6.49), p-dodecylphenol (7.94), 1,4 cyclohexylenedimethylenebis(2-ethylhexanoate) (8.14), trioctylphosphineoxide (9.74), oleylalcohol (7.69), 2-hexyl-1-decanol (7.04), isopropylpalmitate (8.39), dihexylhexylphosphonate (6.32), 2-ethylhexyl-p-hydroxybenzoate (5.56), bis(2-ethylhexyl)azelate (9.38), bis(2-ethylhexyl) sulfoxide (5.77), dioctylamine (6.89), trioctylamine (10.76), dodecylbenzene (8.61), and 1,1-bis(3,4-dimethylphenyl) ethane (7.35).

In accordance with preferred embodiments, the adjacent image forming layer which is closest to the solvent-free yellow image forming layer in the elements of the invention is substantially free of high boiling solvents which have a logP of less than about 5.5. In accordance with especially preferred embodiments, all image forming layers of the elements of the invention are substantially free of high boiling solvents which have a logP of less than about 5.5. In

accordance with most preferred embodiments, all hydrophilic colloid layers on the same side of the support as the solvent-free yellow image forming layer in the elements of the invention are substantially free of high boiling solvents which have a logP of less than 5.5.

Multicolor photographic elements in accordance with preferred embodiments of the invention preferably comprise a support bearing light sensitive image dye forming layers sensitized to the blue (approx. 380–500 nm), green (approx. 500–600 nm), and red (approx. 600–760 nm) regions of the electromagnetic spectrum. In accordance with a preferred embodiment of the invention, the element comprises cyan, magenta and yellow dye forming silver halide emulsion hydrophilic colloid layer units sensitized to the red, green and blue regions of the spectrum. Each unit can comprise a single emulsion layer or multiple emulsion layers sensitive to a given region of the spectrum. The layers of the element, including the layers of the image forming units, can be arranged in various orders as known in the art. It is within the scope of this invention, however, for the light sensitive material to alternatively or additionally be sensitive to one or more regions of the electromagnetic spectrum outside the visible, such as the infrared region of the spectrum. In most color photographic systems, color-forming couplers are incorporated in the light-sensitive photographic emulsion layers so that during development, they are available in the emulsion layer to react with the color developing agent that is oxidized by silver halide image development. Non-diffusing couplers are incorporated in photographic emulsion layers. When the dye image formed is to be used in situ, couplers are selected which form non-diffusing dyes. Color photographic systems can also be used to produce black-and-white images from non-diffusing couplers as described, e.g., by Edwards et al. in International Publication No. WO 93/012465.

The invention is particularly useful with color photographic print elements, and especially to photographic print elements designed for exposure through a negative film and projection display, such as motion picture print and intermediate films. In color photographic element printing, there are usually three records to record in the image area frame region of a print film, i.e., red, green and blue. The original record to be reproduced is preferably an image composed of sub-records having radiation patterns in different regions of the spectrum. Typically it will be a multicolor record composed of sub-records formed from cyan, magenta and yellow dyes. The principles by which such materials form a color image are described in James, *The Theory of the Photographic Process*, Chapter 12, *Principles and Chemistry of Color Photography*, pp 335–372, 1977, Macmillan Publishing Co. New York, and suitable materials useful to form original records are described in *Research Disclosure*, December, 1987, Item 17643, published by Industrial Opportunities Ltd., Homewell Havant, Hampshire, P09 1EF, United Kingdom, and *Research Disclosure*, September 1994, Item 36544, published by Kenneth Mason Publications, Ltd., Emsworth, Hampshire PO10 7DQ, England. Materials in which such images are formed can be exposed to an original scene in a camera, or can be duplicates formed from such camera origination materials, e.g., records formed in color negative intermediate films such as those identified by the tradenames Eastman Color Intermediate Films 2244, 5244 and 7244. Alternatively, the original record may be in the form of electronic image data, which may be used to control a printer apparatus, such as a laser printer, for selective imagewise exposure of a print film in accordance with the invention.

Image dyes formed in photographic print elements designed for direct or projection viewing generally have been found to be far more susceptible to degradation due to light exposures than dyes formed in camera negative films, which are typically stored in dark conditions. Accordingly, the photographic elements of the invention in accordance with particular embodiments of the invention preferably comprise photographic print elements. Relatively small grain, high chloride emulsions (e.g., emulsions having average grain size equivalent circular diameters of less than about 1 micron and halide contents of greater than 50 mole % chloride) are typically used in photographic print films and papers in order to optimize print image quality and enable rapid processing. Such emulsions typically result in relatively low speed photographic elements in comparison to camera negative films. Low speed is compensated for by the use of relatively high intensity print lamps or lasers for exposing such print elements. For comparison purposes, it is noted that print films and papers, such as motion picture color print films, e.g., when rated using the same international standards criteria used for rating camera negative films, would typically have an ISO speed rating of less than 10, which is several stops slower than the slowest camera negative films in current use.

In the following discussion of suitable materials for use in the emulsions and elements that can be used in conjunction with the invention, reference will be made to *Research Disclosure*, September 1994, Item 36544, available as described above, which will be identified hereafter by the term "*Research Disclosure*." The contents of the *Research Disclosure*, including the patents and publications referenced therein, are incorporated herein by reference, and the Sections hereafter referred to are Sections of the *Research Disclosure*, Item 36544.

Suitable silver halide emulsions and their preparation as well as methods of chemical and spectral sensitization are described in Sections I, and III–IV. Vehicles and vehicle related addenda are described in Section II. Dye image formers and modifiers are described in Section X. Various additives such as UV dyes, brighteners, luminescent dyes, antifoggants, stabilizers, light absorbing and scattering materials, coating aids, plasticizers, lubricants, antistats and matting agents are described, for example, in Sections VI–IX. Layers and layer arrangements, color negative and color positive features, scan facilitating features, supports, exposure and processing conditions can be found in Sections XI–XX.

The solvent-free yellow image forming layers of the photographic elements of the invention may advantageously be used in combination with solid substituted bisphenol light stabilizers as disclosed in concurrently filed, commonly assigned copending U.S. patent application Ser. No. 08/916, 882 (Kodak Docket 75629AJA) incorporated by reference above.

It is also contemplated that the materials and processes described in an article titled "Typical and Preferred Color Paper, Color Negative, and Color Reversal Photographic Elements and Processing," published in *Research Disclosure*, February 1995, Item 37038 also may be advantageously used with elements of the invention.

Photographic light-sensitive print elements of the invention may utilize silver halide emulsion image forming layers wherein chloride, bromide and/or iodide are present alone or as mixtures or combinations of at least two halides. The combinations significantly influence the performance characteristics of the silver halide emulsion. Print elements are typically distinguished from camera negative elements by

the use of high chloride (e.g., greater than 50 mole % chloride) silver halide emulsions containing no or only a minor amount of bromide (typically less than 40 mole %), which are also typically substantially free of iodide. As explained in Atwell, U.S. Pat. No. 4,269,927, silver halide with a high chloride content possesses a number of highly advantageous characteristics. For example, high chloride silver halides are more soluble than high bromide silver halide, thereby permitting development to be achieved in shorter times. Furthermore, the release of chloride into the developing solution has less restraining action on development compared to bromide and iodide and this allows developing solutions to be utilized in a manner that reduces the amount of waste developing solution. Since print films are intended to be exposed by a controlled light source, the imaging speed gain which would be associated with high bromide emulsions and/or iodide incorporation offers little benefit for such print films.

Photographic print elements are also distinguished from camera negative elements in that print elements typically comprise only fine silver halide emulsions comprising grains having an average equivalent circular diameter (ECD) of less than about 1 micron, where the ECD of a grain is the diameter of a circle having the area equal to the projected area of a grain. The ECDs of silver halide emulsion grains are usually less than 0.60 micron in red and green sensitized layers and less than 0.90 micron in blue sensitized layers of a color photographic print element. Such fine grain emulsions used in print elements generally have an aspect ratio of less than 1.3, where the aspect ratio is the ratio of a grain's ECD to its thickness. Such grains may take any regular shapes, such as cubic, octahedral or cubo-octahedral (i.e., tetradecahedral) grains, or the grains can take other shapes attributable to ripening, twinning, screw dislocations, etc. Typically, print element emulsions grains are bounded primarily by {100} crystal faces, since {100} grain faces are exceptionally stable. Specific examples of high chloride emulsions used for preparing photographic prints are provided in U.S. Pat. Nos. 4,865,962; 5,252,454; and 5,252,456, the disclosures of which are here incorporated by reference.

The yellow, cyan and magenta dye forming couplers that may be used in the elements of the invention can be defined as being 4-equivalent or 2-equivalent depending on the the number of atoms of  $\text{Ag}^+$  required to form one molecule of dye. A 4-equivalent coupler can generally be converted into a 2-equivalent coupler by replacing a hydrogen at the coupling site with a different coupling-off group. Coupling-off groups are well known in the art. Such groups can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like. Representative classes of such coupling-off groups include, for example, chloro, alkoxy, aryloxy, hetero-oxy, sulfonyloxy, acyloxy, acyl, heterocycl, sulfonamido, mercaptotetrazole, benzothiazole, alkylthio (such as mercaptopropionic acid), arylthio, phosphoryloxy and arylazo. These coupling-off groups are described in the art, for example, in U.S. Pat. Nos. 2,455,169; 3,227,551; 3,432,521; 3,476,563; 3,617,291; 3,880,661; 4,052,212 and 4,134,766; and in U.K. Patents and published Application Nos. 1,466,728; 1,531,927; 1,533,039; 2,006,755A and 2,017,704A, the disclosures of which are incorporated herein by reference.

Image dye forming couplers may be included in elements of the invention such as couplers that form cyan dyes upon reaction with oxidized color developing agents which are described in such representative patents and publications as: U.S. Pat. Nos. 2,367,531; 2,423,730; 2,474,293; 2,772,162; 2,895,826; 3,002,836; 3,034,892; 3,041,236; 4,883,746 and "Farbkuppler—Eine Literature Übersicht," published in Agfa Mitteilungen, Band III, pp. 156-175 (1961). Preferably such couplers are phenols and naphthols that form cyan dyes on reaction with oxidized color developing agent. Also preferable are the cyan couplers described in, for instance, European Patent Application Nos. 544,322; 556,700; 556,777; 565,096; 570,006; and 574,948.

Typical cyan couplers are represented by the following formulas:



wherein R<sub>1</sub> and R<sub>5</sub> each represent a hydrogen or a substituent; R<sub>2</sub> represents a substituent; R<sub>3</sub> and R<sub>4</sub> each represent an electron attractive group having a Hammett's substituent constant  $s_{para}$  of 0.2 or more and the sum of the  $s_{para}$  values of R<sub>3</sub> and R<sub>4</sub> is 0.65 or more; R<sub>6</sub> represents an electron attractive group having a Hammett's substituent constant  $s_{para}$  of 0.35 or more; X represents a hydrogen or a coupling-off group; Z<sub>1</sub> represents nonmetallic atoms necessary for forming a nitrogen-containing, six-membered, heterocyclic ring which has at least one dissociative group. A dissociative group has an acidic proton, e.g. —NH—, —CH(R)—, etc., that preferably has a pKa value of from 3 to 12 in water. The values for Hammett's substituent constants can be found or measured as is described in the literature. For example, see C. Hansch and A. J. Leo, *J. Med. Chem.*, 16, 1207 (1973); *J. Med. Chem.*, 20, 304 (1977); and J. A. Dean, *Lange's Handbook of Chemistry*, 12th Ed. (1979) (McGraw-Hill).

More preferable are cyan couplers of the following formulas:



wherein R<sub>7</sub> represents a substituent (preferably a carbamoyl, ureido, or carbonamido group); R<sub>8</sub> represents a substituent (preferably individually selected from halogen, alkyl, and carbonamido groups); R<sub>9</sub> represents a ballast substituent; R<sub>10</sub> represents a hydrogen or a substituent (preferably a carbonamido or sulphonamido group); X represents a hydrogen or a coupling-off group; and m is from 1-3. Couplers of the structure CYAN-7 are most preferable for use in elements of the invention.

Couplers that form magenta dyes upon reaction with oxidized color developing agent which can be incorporated in elements of the invention are described in such representative patents and publications as: U.S. Pat. Nos. 2,600,788; 2,369,489; 2,343,703; 2,311,082; 2,908,573; 3,062,653; 3,152,896; 3,519,429 and "Farbkuppler—Eine Literature Ubersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents. Especially preferred couplers are 1H-pyrazolo [5,1-c]-1,2,4-triazole and 1H-pyrazolo [1,5-b]-1,2,4-triazole. Examples of 1H-pyrazolo [5,1-c]-1,2,4-triazole couplers are described in U.K. Patent Nos. 1,247,493; 1,252,418; 1,398, 979; U.S. Pat. Nos. 4,443,536; 4,514,490; 4,540,654; 4,590, 153; 4,665,015; 4,822,730; 4,945,034; 5,017,465; and 5,023,170. Examples of 1H-pyrazolo [1,5-b]-1,2,4-triazoles can be found in European Patent Applications 176,804; 177,765; U.S. Pat. Nos. 4,659,652; 5,066,575; and 5,250, 400.

Typical pyrazoloazole and pyrazolone couplers are represented by the following formulas:



MAGENTA-1



MAGENTA-2

wherein R<sub>a</sub> and R<sub>b</sub> independently represent H or a substituent; R<sub>c</sub> is a substituent (preferably an aryl group); R<sub>d</sub> is a substituent (preferably an anilino, carbonamido, ureido, carbamoyl, alkoxy, aryloxycarbonyl, alkoxy carbonyl, or N-heterocyclic group); X is hydrogen or a coupling-off group; and Z<sub>a</sub>, Z<sub>b</sub>, and Z<sub>c</sub> are independently a substituted methine group, =N=, =C=, or —NH—, provided that one of either the Z<sub>a</sub>—Z<sub>b</sub> bond or the Z<sub>b</sub>—Z<sub>c</sub> bond is a double bond and the other is a single bond, and when the

## CYAN-7

Z<sub>b</sub>—Z<sub>c</sub> bond is a carbon—carbon double bond, it may form part of an aromatic ring, and at least one of Z<sub>a</sub>, Z<sub>b</sub>, and Z<sub>c</sub> represents a methine group connected to the group R<sub>b</sub>. Use of yellow image forming layers in accordance with the invention may be particularly useful in combination with magenta image forming layers comprising pyrazoloazole dye forming couplers of formula MAGENTA-1 to provide improved color reproduction performance.

Typical examples of photographic substituents which may be included in the yellow, cyan and magenta couplers which may be used in the elements of the invention include alkyl, aryl, anilino, carbonamido, sulfonamido, alkylthio, arylthio, alkenyl, cycloalkyl, and further to these exemplified are halogen, cycloalkenyl, alkynyl, heterocycl, sulfonyl, sulfinyl, phosphonyl, acyl, carbamoyl, sulfamoyl, cyano, alkoxy, aryloxy, heterocyclyloxy, siloxy, acyloxy, carbamoyloxy, amino, alkylamino, imido, ureido, sulfamoyl amino, alkoxy carbonyl amino, aryloxycarbonyl amino, alkoxy carbonyl, aryloxycarbonyl, heterocyclylthio, spiro compound residues and bridged hydrocarbon compound residues. Usually the substituent will have less than 30 carbon atoms and typically less than 20 carbon atoms. It is understood throughout this specification that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form, but also its form substituted with any other photographically useful substituents.

To control the migration of various components coated in a photographic layer, including couplers, it may be desirable to include a high molecular weight hydrophobe or "ballast" group in the component molecule. Representative ballast groups include substituted or unsubstituted alkyl or aryl groups containing 8 to 40 carbon atoms. Representative substituents on such groups include alkyl, aryl, alkoxy, aryloxy, alkylthio, hydroxy, halogen, aryloxycarbonyl, aryloxycarbonyl, carboxy, acyl, acyloxy, amino, anilino, carbonamido (also known as acylamino), carbamoyl, alkylsulfonyl, arylsulfonyl, sulfonamido, and sulfamoyl groups wherein the substituents typically contain 1 to 40 carbon atoms. Such substituents can also be further substituted. Alternatively, the molecule can be made immobile by attachment to a polymeric backbone.

It may be useful to use a combination of couplers any of which may contain known ballasts or coupling-off groups such as those described in U.S. Pat. Nos. 4,301,235; 4,853, 319 and 4,351,897.

If desired, the photographic element can be used in conjunction with an applied magnetic layer as described in Research Disclosure, November 1992, Item 34390. It is also specifically contemplated to use photographic elements according to the invention in combination with technology useful in small format film as described in Research Disclosure, June 1994, Item 36230. Research Disclosure is published by Kenneth Mason Publications, Ltd., Dudley House, 12 North Street, Emsworth, Hampshire P010 7DQ, ENGLAND.

Photographic elements in accordance with the invention may comprise any conventional support materials, which may be reflective or transparent. Preferred supports for elements in accordance with the invention comprise transparent polymeric films, such as cellulose nitrate and cellulose esters (such as cellulose triacetate and diacetate), polycarbonate, and polyesters of dibasic aromatic carboxylic acids with divalent alcohols such as poly(ethylene terephthalate). In addition to the light sensitive image forming layers described above, the photographic elements of the

## 13

invention may include further features and layers as are known in the art, including, e.g., antistatic, antihalation, subbing, interlayer, backing, and overcoat layers. Polyester supports, e.g., typically employ undercoat or primer layers to improve adhesion of other layers thereto. Such undercoat layers are well known in the art and comprise, e.g., a vinylidene chloride/methyl acrylate/itaconic acid terpolymer or vinylidene chloride/acrylonitrile/acrylic acid terpolymer as described in U.S. Pat. Nos. 2,627,088; 2,698,235; 2,698,240; 2,943,937; 3,143,421; 3,201,249; 3,271,178; 3,501,301.

Photographic elements of the invention preferably comprise an antihalation layer comprising process removable filter dyes or silver. The antihalation layer may be located between the light sensitive layers and the support, or may be positioned on the back side of the support opposite to the light sensitive layers. The filter dyes and/or silver used in antihalation layers are preferably designed to be solubilized and removed or decolorized during photographic processing. Conventional processing of photographic print elements include the Kodak ECP-2B Process for motion picture print films, described in Kodak Publication No. H-24, Manual For Processing Eastman Color Films, the disclosure of which is hereby incorporated by reference.

The following examples illustrate the preparation of photographic elements in accordance with this invention.

## EXAMPLE 1

80.0 g of cyan coupler C-1 was dissolved in 96.0 g of tricresylphosphate (S-1) and 80.0 g of ethyl acetate at 70° C. This oil phase solution was then combined with an aqueous phase solution consisting of 80.0 g gelatin, 60.0 g of a 10% solution of Alkanol-XC (Dupont), and 604.0 g of distilled water. This mixture was then passed through a Gaulin colloid mill five times followed by removal of ethyl acetate by rotary evaporation. Distilled water was then added back to form Dispersion A which consisted of 8.0% coupler and 8.0% gel. Dispersions B through G were similarly prepared using alternative solvents instead of S-1 as described in Table I. Dispersion H was also prepared similarly, except that no permanent coupler solvent was employed and 176.0 g of ethyl acetate was used.

Dispersion A was incorporated in a multilayer photographic element (element 1) by coating the following layers on a gelatin subbed polyethylene terephthalate support with a rem-jet carbon black containing backing layer. The yellow image forming layer (Blue Light Sensitive Layer 1) coating composition was free of high boiling permanent solvent, the yellow dye forming coupler Y-1 being dispersed in the form of a permanent solvent-free evaporated dispersion.

## Layer 1: Blue Light Sensitive Layer

AgCl cubic grain emulsion, 0.58 micron, spectrally sensitized with SD-1, 0.3336 mmole/Ag mole, 645.6 mg/sq. m.

AgCl cubic grain emulsion, 0.76 micron, spectrally sensitized with SD-1, 0.2669 mmole/Ag mole, 215.2 mg/sq. m.

Yellow dye forming coupler (Y-1), 1291.2 mg/sq. m.

Sequestrant cpd (SQ-1), 305.8 mg/sq. m.

Sequestrant cpd (SQ-2), 100.0 mg/sq. m.

Gelatin, 2797.6 mg/sq. m.

Spreading aids.

## Layer 2: Interlayer

Oxidized developer scavenger (SC-1), 75.3 mg/sq. m.

Gelatin, 645.6 mg/sq. m.

Spreading aids.

## Layer 3: Red Light Sensitive Layer

AgClBr cubic grain emulsion, 25% Br, 0.15 micron, spectrally sensitized with SD-2, 0.1808 mmole/Ag mole,

## 14

supersensitizer compound (SS-1), 0.6327 mmole/Ag mole, 397.0 mg/sq. m.

AgClBr cubic grain emulsion, 25% Br, 0.24 micron, spectrally sensitized with SD-2, 0.1356 mmole/Ag mole, supersensitizer compound (SS-1), 0.7444 mmole/Ag mole, 44.1 mg/sq. m.

Cyan dye forming coupler (C-1) from Dispersion A, 914.6 mg/sq. m.

Coupler Solvent (S-1), 1097.5 mg/sq. m.

Oxidized developer scavenger (SC-1), 12.9 mg/sq. m.

Gelatin, 3410.9 mg/sq. m.

Spreading aids.

## Layer 4: Interlayer

Oxidized developer scavenger (SC-1), 75.3 mg/sq. m.

Gelatin, 645.6 mg/sq. m.

Spreading aids.

## Layer 5: Green Light Sensitive Layer

AgClBr cubic grain emulsion, 25% Br, 0.15 micron, spectrally sensitized with SD-3, 0.5273 mmole/Ag mole, supersensitizer compound (SS-1), 1.1212 mmole/Ag mole, 419.6 mg/sq. m.

AgClBr cubic grain emulsion, 25% Br, 0.24 micron, spectrally sensitized with SD-3, 0.4785 mmole/Ag mole, supersensitizer compound (SS-1), 1.3902 mmole/Ag mole, 32.3 mg/sq. m.

Magenta dye forming coupler (M-1), 645.6 mg/sq. m.

Oxidized developer scavenger (SC-1), 53.8 mg/sq. m.

Gelatin, 1915.3 mg/sq. m.

Spreading aids.

## Layer 6: Protective Overcoat Layer

Poly (dimethyl siloxane) 200-CS, 65.9 mg/sq. m.

Poly (methyl methacrylate) beads, 5.0 mg/sq. m.

Gelatin, 977.0 mg/sq. m.

Soluble green absorber dye (AD-1), 32.3 mg/sq. m.

Soluble green absorber dye (AD-2), 32.3 mg/sq. m.

Soluble blue absorber dye (AD-3), 16.1 mg/sq. m.

Soluble red absorber dye (AD-4), 110.8 mg/sq. m.

Gelatin hardener.

Spreading aids.

Dispersions B through H were similarly incorporated into the previously described photographic element as elements 2 through 8, respectively, as described in Table I.

Dispersions A through H were also incorporated into another photographic element similar to that previously described except that 322.8 mg/sq. m. of light stabilizer ST-1 was included in the blue light sensitive layer.

The elements were exposed for 1/500 second by means of a 3000K Tungsten light source through a 0-3 neutral density step tablet, a heat-absorbing filter, and a filter designed to represent a motion picture color negative film. After exposure, the elements were processed through Process ECP-2B with the exception that those steps specific to sound track development were omitted. The process consisted of a prebath (10"), water rinse (20"), color developer (3'), stop bath (40"), first wash (40"), first fix (40"), second wash (40"), bleach (1'), third wash (40"), second fix (40"), fourth wash (1'), final rinse (10"), and then drying with hot air. The ECP-2B Prebath consists of:

|                                |         |
|--------------------------------|---------|
| Water                          | 800 mL  |
| Borax (decahydrate)            | 20.0 g  |
| Sodium sulfate (anhydrous)     | 100.0 g |
| Sodium hydroxide               | 1.0 g   |
| Water to make 1 liter          |         |
| pH @ 26.7° C. is 9.25 +/- 0.10 |         |

The ECP-2B Color Developer consists of:

|                                                                                                         |         |  |
|---------------------------------------------------------------------------------------------------------|---------|--|
| Water                                                                                                   | 900 mL  |  |
| Kodak Anti-Calcium, No. 4 (40% solution of a pentasodium salt of nitrilo-tri(methylene phosphonic acid) | 1.00 mL |  |
| Sodium sulfite (anhydrous)                                                                              | 4.35 g  |  |
| Sodium bromide (anhydrous)                                                                              | 1.72 g  |  |
| Sodium carbonate (anhydrous)                                                                            | 17.1 g  |  |
| Kodak Color Developing Agent, CD-2                                                                      | 2.95 g  |  |
| Sulfuric acid (7.0N)                                                                                    | 0.62 mL |  |
| Water to make 1 liter                                                                                   |         |  |
| pH @ 26.7° C. is 10.53 +/- 0.05                                                                         |         |  |

The ECP-2B Stop Bath consists of:

|                       |        |  |
|-----------------------|--------|--|
| Water                 | 900 mL |  |
| Sulfuric acid (7.0N)  | 50 mL  |  |
| Water to make 1 liter |        |  |
| pH @ 26.7° C. is 0.90 |        |  |

The ECP-2B Fixer consists of:

|                                       |          |  |
|---------------------------------------|----------|--|
| Water                                 | 800 mL   |  |
| Ammonium thiosulfate (58.0% solution) | 100.0 mL |  |
| Sodium bisulfite (anhydrous)          |          |  |
| Water to make 1 liter                 | 13.0 g   |  |
| pH @ 26.7° C. is 5.00 +/- 0.15        |          |  |

The ECP-2B Ferricyanide Bleach consists of:

|                                |        |  |
|--------------------------------|--------|--|
| Water                          | 900 mL |  |
| Potassium ferricyanide         | 30.0 g |  |
| Sodium bromide (anhydrous)     | 17.0 g |  |
| Water to make 1 liter          |        |  |
| pH @ 26.7° C. is 6.50 +/- 0.05 |        |  |

The Final Rinse solution consists of:

|                               |        |  |
|-------------------------------|--------|--|
| Water                         | 900 mL |  |
| Kodak Photo-Flo 200™ Solution | 3.0 mL |  |
| Water to make 1 liter         |        |  |

Processing of the exposed elements was done with the color developing solution adjusted to 36.7° C. The stopping, fixing, bleaching, washing, and final rinsing solution temperatures were adjusted to 26.7° C.

The optical density due to dye formation was then measured on a densitometer using filters in the densitometer appropriate to the intended use of the photographic element. Dye density was then graphed versus log(exposure) to form the Red, Green, and Blue D-logE characteristic curves of the photographic elements.

The processed elements were then irradiated with light from a high intensity 50 Klux Xenon light source for 3 days. After irradiation, the dye density was measured again as described above. The amount of red, green, and blue density lost due to light fading from an initial density of 1.7 for each element is reported in Table I.

TABLE I

## 3 Day 50 Klux Light Fade Data

| Element   | Cyan       | Cyan    | Yellow Layer | Delta Density |       |       |       |
|-----------|------------|---------|--------------|---------------|-------|-------|-------|
|           | Coupler    | Coupler |              | Red           | Green | Blue  |       |
| No.       | Dispersion | Solvent | Log P        | Components    | Red   | Green | Blue  |
| 1 (Inv)   | A          | S-1     | 6.58         | Y-1           | -0.02 | -0.37 | -0.12 |
| 2 (Comp)  | B          | S-2     | 4.69         | Y-1           | -0.06 | -0.37 | -0.27 |
| 3 (Inv)   | C          | S-3     | 5.98         | Y-1           | -0.07 | -0.37 | -0.14 |
| 4 (Comp)  | D          | S-4     | 4.99         | Y-1           | -0.06 | -0.35 | -0.24 |
| 5 (Comp)  | E          | S-5     | 4.21         | Y-1           | -0.07 | -0.37 | -0.34 |
| 6 (Inv)   | F          | S-6     | 9.49         | Y-1           | -0.07 | -0.38 | -0.15 |
| 7 (Inv)   | G          | S-7     | 11.04        | Y-1           | -0.06 | -0.37 | -0.12 |
| 8 (Comp)  | H          | None    | —            | Y-1           | -0.11 | -0.37 | -0.14 |
| 9 (Inv)   | A          | S-1     | 6.58         | Y-1 + ST-1    | -0.07 | -0.38 | -0.02 |
| 10 (Comp) | B          | S-2     | 4.69         | Y-1 + ST-1    | -0.06 | -0.36 | -0.16 |
| 11 (Inv)  | C          | S-3     | 5.98         | Y-1 + ST-1    | -0.07 | -0.40 | -0.09 |
| 12 (Comp) | D          | S-4     | 4.99         | Y-1 + ST-1    | -0.12 | -0.40 | -0.14 |
| 13 (Comp) | E          | S-5     | 4.21         | Y-1 + ST-1    | -0.13 | -0.42 | -0.26 |
| 14 (Inv)  | F          | S-6     | 9.49         | Y-1 + ST-1    | -0.13 | -0.42 | -0.09 |
| 15 (Inv)  | G          | S-7     | 11.04        | Y-1 + ST-1    | -0.10 | -0.41 | -0.06 |
| 16 (Comp) | H          | None    | —            | Y-1 + ST-1    | -0.12 | -0.43 | -0.08 |

These data clearly show that yellow dye light stability in the blue light sensitive layer with no solvent is degraded

5,879,867

**17**

unless the coupler solvent employed in the adjacent imaging layer (the red light sensitive layer) has a calculated log P value of 5.5 or greater.

solvent S-1



solvent S-2



solvent S-3



solvent S-4



solvent S-5



solvent S-6



solvent S-7

**18**

The following structures represent compounds utilized in the above described photographic elements.

19

20

-continued

green sensitizing dye SD-3



supersensitizer SS-1



magenta coupler M-1



scavenger SC-1



soluble green filter dye AD-1



5,879,867

**21**

**22**

-continued

soluble green filter dye AD-2



red sensitizing dye SD-2



cyan coupler C-1



soluble red filter dye AD-4



blue sensitizing dye SD-1



-continued

yellow coupler Y-1



soluble blue filter dye AD-3



sequestrant SQ-1



sequestrant SQ-2



stabilizer ST-1



This invention has been described in detail with particular reference to preferred embodiments thereof. It will be understood that variations and modifications can be made within the spirit and scope of the invention.

We claim:

1. A silver halide light sensitive photographic element comprising a support bearing at least one yellow image forming hydrophilic colloid layer comprising yellow image dye forming couplers, at least one hydrophilic colloid layer immediately adjacent to the yellow image forming layer, and at least one adjacent cyan or magenta image forming hydrophilic colloid layer comprising cyan or magenta image dye forming couplers; wherein the yellow image forming layer is substantially free of high boiling permanent solvent, the immediately adjacent hydrophilic colloid layers and the

55

adjacent image forming layer are substantially free of high boiling permanent solvents having a logP value of less than about 5.5, and the adjacent image forming layer contains a high boiling permanent solvent having a logP value of at least about 5.5.

2. The element of claim 1, wherein the at least one adjacent image forming layer comprises cyan image dye forming couplers.

3. The element of claim 2, wherein all image forming layers are substantially free of high boiling permanent solvents having a logP value of less than about 5.5.

4. The element of claim 1, wherein the at least one adjacent image forming layer comprises magenta image dye forming couplers.

60

65

5. The element of claim 4, wherein all image forming layers are substantially free of high boiling permanent solvents having a logP value of less than about 5.5.

6. The element of claim 1, wherein the yellow image forming layer comprises a blue-sensitive silver halide emulsion and yellow image dye forming coupler, and the adjacent image forming layer comprises either a cyan image forming layer comprising red-sensitive silver halide emulsion and cyan image dye forming coupler or a magenta image forming layer comprising green-sensitive silver halide emulsion and magenta image dye forming coupler.

7. The element of claim 6, wherein the adjacent image forming layer comprises a cyan image forming layer comprising red-sensitive silver halide emulsion and cyan image dye forming coupler, and further comprising a magenta image forming layer comprising green-sensitive silver halide emulsion and magenta image dye forming coupler.

8. The element of claim 6, wherein the adjacent image forming layer comprises a magenta image forming layer comprising green-sensitive silver halide emulsion and magenta image dye forming coupler, and further comprising a cyan image forming layer comprising red-sensitive silver halide emulsion and cyan image dye forming coupler.

9. The element of claim 1, having an effective ISO speed rating of less than about 10.

10. The element of claim 1, wherein the yellow image forming layer and adjacent image forming layer each comprises silver chloride or bromochloride emulsion grains comprising greater than 50 mole % chloride.

11. The element of claim 10, wherein the emulsion grains have an average equivalent circular diameter of less than 1 micron and an aspect ratio of less than 1.3.

12. A silver halide light sensitive photographic element comprising a support bearing in sequential order on one side thereof at least one yellow image forming hydrophilic colloid layer comprising a blue-sensitive silver halide emulsion and yellow image dye forming coupler, a hydrophilic colloid layer immediately adjacent to the yellow image forming layer, at least one cyan image forming hydrophilic

colloid layer comprising red-sensitive silver halide emulsion and cyan image dye forming coupler, and at least one magenta image forming hydrophilic colloid layer comprising green-sensitive silver halide emulsion and magenta image dye forming coupler; wherein the yellow image forming layer is substantially free of high boiling permanent solvent, the hydrophilic colloid layer immediately adjacent to the yellow image forming layer is substantially free of high boiling permanent solvents having a logP of less than about 5.5, and the cyan image forming layer contains a high boiling permanent solvent having a logP value of at least about 5.5 and is substantially free of high boiling permanent solvents having a logP value of less than about 5.5.

13. The element of claim 12, wherein each of the blue-sensitive, red-sensitive, and green-sensitive silver halide emulsions comprise silver chloride or silver bromochloride emulsion grains comprising greater than 50 mole % chloride.

14. The element of claim 13, wherein each of the red-sensitive and green-sensitive silver halide emulsions comprise emulsion grains having an average equivalent circular diameter of less than 0.60 micron, and the blue-sensitive silver halide emulsion comprises emulsion grains having an average equivalent circular diameter of less than 0.90 micron.

15. The element of claim 12, having an effective ISO speed rating of less than about 10.

16. The element of claim 12, wherein all of the yellow, cyan and magenta image forming layers are substantially free of high boiling permanent solvents having a logP value of less than about 5.5.

17. The element of claim 12, wherein all of the hydrophilic colloid layers on the same side of the support as the yellow image forming layer are substantially free of high boiling permanent solvents having a logP of less than about 5.5.

\* \* \* \* \*